# EUROPEAN PATENT SPECIFICATION

(11) **EP 1 245 844 B1**
(45) Date of publication and mention of the grant of the patent: **02.05.2012**
(21) Application number: 02252346.8
(22) Date of filing: 28.03.2002
(51) Int. Cl.: F16C 13/00, B31F 1/07, B23K 26/00

(54) **Laser engraved embossing roll**
Lasergravierte Prägerolle
Rouleau à gaufrer gravé au laser

(30) Priority: 29.03.2001 US 279869
(43) Date of publication of application: 02.10.2002
(73) Proprietor: Georgia-Pacific Consumer Products LP, Atlanta GA 30303 (US)
(72) Inventor: Schulz, Galyn A., Greenville,WI 54942 (US); Bucholz, William T., Greenville, WI 54942 (US); Hennes, Michael E., Neenah, WI 54956 (US)
(74) Representative: Brown, Fraser Gregory James

(56) References cited:
- EP-A- 0 313 766
- EP-A- 1 216 818
- US-A- 3 707 752
- US-A- 4 324 177
- US-A- 4 361 085
- US-A- 5 356 364
- US-A- 5 387 172
- US-A- 5 753 165

## Description

### Field of the Invention

This application claims the right to priority under 35 U.S.C.§ 119(e) based on Provisional Patent Application No. 60/279,869 filed March 29,2001.

The present invention relates to an emboss roll for continuously embossing a moving web of material, such as paper. More particularly, the present invention relates to a laser engravable roll having improved wear characteristics. Still more particularly, the present invention relates to rolls that are patternable by laser engraving techniques that have improved hardness and durability. Finally, the present invention relates to an laser engraved roll made from an epoxy based resin.

### Background of the Invention

The present invention relates to apparatus used to emboss paper products, preferably elongate webs used to make paper goods, e.g., paper towels, toilet tissue, or paper napkins. Embossing is the act of mechanically working a substrate to cause the substrate to conform under pressure to the depths and contours of a patterned embossing roll. Generally, the web is passed between a pair of emboss rolls that, under pressure, form contours within the surface of the paper.

In most configurations at least one of the two roller surfaces directly carries the pattern to be transferred to the paper web. Known configurations include rigid-to-resilient embossing and rigid-to-rigid embossing. The present invention is an improved embossing roll for use in any known embossing configuration.

In a rigid-to-resilient embossing system, a single or multi-ply substrate is passed through a nip formed between a roll whose substantially rigid surface contains the embossing pattern as a multiplicity of protuberances and/or depressions arranged into an aesthetically-pleasing manner, and a second roll, whose substantially resilient surface can be either smooth or also contain a multiplicity of protuberances and/or depressions which cooperate with the rigid surfaced patterned roll. Heretofore, rigid rolls were generally formed from a steel body which is either directly engraved upon or which can contain a hard rubber-covered surface (directly coated or sleeved) upon which the embossing pattern is laser engraved. While a steel roll that has been directly engraved has a longer lifespan, the production of a directly engraved steel roll can require a significant lead time. Known laser engraved sleeves can take less time to make but have a lifespan which is substantially less than that of a steel roll.

Resilient rolls may consist of a steel core directly coated or sleeved with a resilient material and may or may not be engraved with a pattern. If a pattern is present, it may be either a mated or a non-mated pattern with respect to the pattern carried on the rigid roll.

In the rigid-to-rigid embossing process, a single-ply or multi-ply substrate is passed through a nip formed between two substantially rigid rolls. The surfaces of both rolls contain the pattern to be embossed as a multiplicity of protuberances and/or depressions arranged into an aesthetically-pleasing manner where the protuberances and/or depression in the second roll cooperate with those patterned in the first rigid roll. The first rigid roll is generally formed from a steel body which is either directly engraved upon or which can carry a hard rubber-covered surface (directly coated or sleeved) upon which the embossing pattern is laser engraved. The second rigid roll is generally formed from a steel body which is also directly engraved upon or which can carry a hard rubber covered surface (directly coated or sleeved) upon which a matching or mated pattern is conventionally engraved or laser engraved. Laser engravable rolls are known, see for example U.S. patent Nos. 4,211,743 and 5,356,364.

Prior art embossing systems where the embossing pattern is carried directly by one or both of the steel embossing rolls suffer from a number of disadvantages. Specifically, to directly engrave steel can require a significant amount of lead time. Laser engraving of hard rubber has improved the lead time, but has not replaced directly engraved steel rolls due to issues associated with wear. Furthermore, directly engraved steel rolls run the risk that if the emboss pattern gets damaged and a new roll must be produced, the preparation of a new steel roll can require significant time, possibly resulting in machine down time and definitely resulting in increased expense.

The present invention overcomes the disadvantages associated with prior art steel rolls and further addresses the wear issues associated with prior art rubber rolls and sleeves. The present invention provides an embossing roll made from a material that can be patterned and which provides improved wear characteristics. The present invention further provides a resin based roll that is capable of being laser engraved and which exhibits improved wear characteristics and life span in commercial use.

### SUMMARY OF THE INVENTION

In accordance with the invention, there is disclosed a laser engraved embossing roll comprising a laser engraved resin based material which exhibits improved wear resistance wherein the resin material has a Shore D hardness of at least 90. There is further disclosed a laser engraved embossing roll comprising a laser engraved resin material comprising a Bisphenol A epoxy based resin, epichlorohydrin and a filler material wherein the Bisphenol A epoxy based resin has a Shore D hardness of at least 90.

There is still further disclosed, a laser engraved embossing roll comprising a phenolic or styrene based resin that is first patterned and then cured.

Finally, there is disclosed a method of making a patterned web comprising, passing the web between one or more resin based laser engraved embossing rolls.

Additional objects and advantages of the invention will be set forth in part in the description which follows, and in part will be obvious from the description, or may be learned by practice of the invention. The objects and advantages of the invention will be realized and attained by means of the elements and combinations particularly pointed out in the appended claims.

It is to be understood that both the foregoing general description and the following detailed description are exemplary and explanatory only and are not restrictive of the invention, as claimed.

The accompanying drawings, which are incorporated in and constitute a part of this specification, illustrate one embodiment of the invention and together with the description, serve to explain the principles of the invention.

### BRIEF DESCRIPTION OF THE DRAWINGS

Figure 1 is an infrared spectrum of one epoxy resin for use according to the present invention.

Figure 2 is thermogram of one epoxy resin for use according to the present invention.

Figure 3 is a pyrolysis GC/MS chromatogram of one epoxy resin for use according to the present invention.

Figure 4 illustrates an emboss pattern that may be used with the present invention.

### DESCRIPTION OF THE EMBODIMENTS

Reference will now be made in detail to the present embodiments (exemplary embodiments) of the invention, an example of which is illustrated in the accompanying drawings.

The present invention relates to the production of rolls for use in the embossing of elongate webs of material, such as paper and the like. More specifically, the present invention relates to embossing rolls that have improved wear resistant surfaces.

The embossing roll according to the present invention can be either formed from a single laser engraved resin material having a Shore D hardness of at least 90 upon which an embossing pattern is engraved or can be a rigid core that is coated or sleeved with an improved laser engraved resin material having a Shore D hardness of at least 90.

One advantage associated with the present invention is the improvements in production time that may be achieved when the embossing pattern is created using laser engraving. As described above, the pattern can be carried directly by a core material that can be laser engraved or can be present in a sleeve or coating of laser engraved material that surrounds a structurally rigid core.

The core may be produced from any art recognized material which can be sleeved or coated with a laser engraved material. Appropriate materials to produce a structurally rigid core will be readily apparent to the skilled artisan. According to one embodiment of the invention, the core would be steel. Appropriate methods for forming a patternable coating or sleeve over a rigid core include any art recognized method and would be readily apparent to the skilled artisan. Preferred coating methods include dip coating, casting or vulcanizing. Appropriate core preparation may include pretreatment to achieve the necessary adherence between the core and the coating. Pretreatments may include, but are not limited to, sandblasting, sanding, and chemical pretreatment.

Materials for use in the production of rolls according to the present invention are selected from resin materials that are capable of being laser engraved, while exhibiting sufficient hardness that they will withstand the ordinary use conditions of commercial embossing. Prior art rubber rolls having a Shore A hardness on the order of 98 can withstand commercial runs conditions for only about 25 days.

Patternable materials that may be used with the present invention include hard resin based materials. Prior art rubber sleeves are generally at about 99 Shore A hardness and below. The material for use according to the present invention exceeds the 100 Shore A hardness associated with the scale. The materials according to the present invention would reside on the Shore D scale. In the present invention, the material has a Shore D hardness of at least 90.

Preferred materials according to the present invention will not exhibit any substantial wear when used in a standard commercial environment for a least about 3 months, more preferably at least about 6 months, still more preferably at least about 9 months, and most preferably at least about 1 year. The materials according to the present invention can sustain no substantial wear over a 3 to 5 year period. Substantial wear as used in the present invention refers to wear that is at 10 microns or less. Preferred materials according to the present invention will not exhibit wear that is visible to the naked eye at the end of 6, 9 or 12 months from the inception of commercial use.

While resins have not generally been used for embossing rolls, resins provide good durability, good castability, good core adhesion, good printability and good engravability. Appropriate resins would include, but are not limited to, epoxy resins, phenolic resins, isocyanate resins, styrenated resins, polyester resins, thermosetting resins, and polycarbonate resins.

In one embodiment of the present invention, materials for use in the present invention are selected from epoxy based resins, more particularly, epoxy based materials containing Bisphenol A and more preferably containing epichlorohydrin. One preferred material for use according to the present invention has been analyzed and the results of that analysis are set forth in Figures 1-3. Figure 1 is an Infrared spectrum showing that the preferred material according to the present invention is a Bisphenol A type epoxy resin. This preferred material is available from Voith Sulzer under the tradename TOP ROCK. Figure 2 is a thermogram of the TOP ROCK material between 50° C and 800° C. The thermogram was used to determine the temperature at which the chromatogram of Figure 3 was to be carried out. Specifically, this analysis can be used to determine if a material will produce volatiles making it unacceptable for laser engraving. As can be seen from Figure 3, the most significant volatile produced was benzyl alcohol. In addition, decompositions products as seen in Figure 3 included acetone, tetrahydrofuran, toluene, 2-propene-1-ol, 1-butanol, pyridine and alkyl substituted pyridines, acetic acid, benzaldehyde and alkyl substituted phenols.

In an alternative embodiment according to the present invention, the resin may be selected from a material which exhibits characteristics making it capable of being laser engraved prior to heat setting or curing. In this embodiment, a soft resin roll may be patterned through laser engraving. The resin is then cured or heat set to result in a hard material capable of withstanding the pressures associated with commercial embossing. Appropriate resins for use according to this embodiment include phenolic resins and isocyanate resins.

Resin materials for use in the present invention may be filled or unfilled materials. The resin may include up to 50% filler, more preferably less than about 40% filler, most preferably less than about 30% filler. Appropriate resins will be readily apparent to the skilled artisan. Filler materials may be selected from any art recognized fillers.

### Example

An embossing roll was produced from TOP ROCK material obtained from Voith Sulzer. The TOP ROCK roll was laser engraved using the pattern of Figure 4. Top Rock exhibits a Shore D hardness of 91.

## Claims

1. A laser engraved embossing roll comprising a laser engraved resin material having a Shore D hardness of at least 90.

2. The embossing roll of Claim 1, wherein the resin Is chosen from at least one of epoxy resins, phenolic resins, isocyanate resins, styrenated resins, polyester resins, thermosetting resins and polycarbonate resins.

3. The embossing roll of Claim 2, wherein the resin material is chosen from at least one epoxy resin.

4. The embossing roll of Claim 3, wherein the epoxy resin is a Bisphenol A resin.

5. The embossing roll of Claim 3 or 4, further comprising epichlorohydrin.

6. The embossing roll of any of claims 1 to 5, further comprising a filler.

7. The embossing roll of Claim 6, wherein the filler is present in an amount of less than 50%.

8. The embossing roll of Claim 7, wherein the filler is present in an amount of less than 30%.

9. The embossing roll of any preceding claim, wherein the resin material forms both the roll surface and the roll core.

10. The embossing roll of any preceding claim, wherein the resin material forms the roll surface and wherein the roll contains a rigid core of another material.

11. The embossing roll of claim 10, wherein the core is steel.

12. A method of producing a laser engraved embossing roll comprising:
providing a roll having a surface of a laser engravable resin material which will provide a Shore D hardness of at least 90 for the final roll; and
laser engraving the resin material to establish an embossing pattern in the surface.

13. The method according to Claim 12, further comprising heat setting or curing the resin material after the embossing pattern has been established.

14. The method of Claim 12 or 13, wherein the resin surface is formed over a steel core.

15. The method of Claim 14, wherein the resin surface is produced by dip coating, casting or vulcanizing.

16. The method of Claim 14 or 15, wherein the steel core is treated by one or more of sandblasting, sanding or chemical pretreatment prior to providing the resin surface over the core.

17. The method according to any of claims 12 to 16 wherein the resin is chosen from at least one of epoxy resins, phenolic resins, isocyanate resins, styrenated resins, polyester resins, thermosetting resins and polycarbonate resins.

18. The method according to any of claims 12 to 17, wherein the resin material is chosen from at least one epoxy resin.

19. The method according to Claim 18, wherein the epoxy resin is a Bisphenol A resin.

20. The method according to any of claims 12 to 19, the resin material further comprising epichlorohydrin.

21. The method according to any of claims 12 to 20, the resin material further comprising a filler.

22. The method according to Claim 21, wherein the filler is present in an amount of less than 50%.

23. The method according to Claim 22, wherein the filler is present in an amount of less than 30%.

## Patentansprüche

1. Lasergravierte Prägewalze, umfassend ein lasergraviertes Harzmaterial, das eine Shore-Härte D von mindestens 90 aufweist.

2. Prägewalze nach Anspruch 1, wobei das Harz aus mindestens einem von Epoxidharzen, Phenolharzen, Isocyanatharzen, Styrolharzen, Polyesterharzen, Duroplastharzen und Polycarbonatharzen ausgewählt wird.

3. Prägewalze nach Anspruch 2, wobei das Harzmaterial aus mindestens einem Epoxidharz ausgewählt wird.

4. Prägewalze nach Anspruch 3, wobei das Epoxidharz ein Bisphenol-A-Harz ist.

5. Prägewalze nach Anspruch 3 oder 4, ferner umfassend Epichlorhydrin.

6. Prägewalze nach einem der Ansprüche 1 bis 5, ferner umfassend einen Füllstoff.

7. Prägewalze nach Anspruch 6, wobei der Füllstoff in einer Menge von weniger als 50 % vorliegt.

8. Prägewalze nach Anspruch 7, wobei der Füllstoff in einer Menge von weniger als 30 % vorliegt.

9. Prägewalze nach einem der vorhergehenden Ansprüche, wobei das Harzmaterial sowohl die Walzenoberfläche als auch den Walzenkern bildet.

10. Prägewalze nach einem der vorhergehenden Ansprüche, wobei das Harzmaterial die Walzenoberfläche bildet, und wobei die Walze einen unbiegsamen Kern aus einem anderen Material enthält.

11. Prägewalze nach Anspruch 10, wobei der Kern Stahl ist.

12. Verfahren zum Fertigen einer lasergravierten Prägewalze, umfassend folgende Schritte:
Bereitstellen einer Walze, die eine Oberfläche aus einem lasergravierten Harzmaterial aufweist, das eine Shore-Härte D von mindestens 90 für die fertige Walze bereitstellt; und
Lasergravieren des Harzmaterials, um ein Prägemuster an der Oberfläche zu erstellen.

13. Verfahren nach Anspruch 12, ferner umfassend das Thermofixieren oder Aushärten des Harzmaterials, nachdem das Prägemuster erstellt wurde.

14. Verfahren nach Anspruch 12 oder 13, wobei die Harzoberfläche über einem Stahlkern gebildet ist.

15. Verfahren nach Anspruch 14, wobei die Harzoberfläche durch Tauchverfahren, Gießen oder Vulkanisieren erzeugt wird.

16. Verfahren nach Anspruch 14 oder 15, wobei der Stahlkern durch eines oder mehreres von Sandstrahlen, Schmirgeln oder chemischer Vorbehandlung vor dem Bereitstellen der Harzoberfläche über dem Kern behandelt wird.

17. Verfahren nach einem der Ansprüche 12 bis 16, wobei das Harz aus mindestens einem von Epoxidharzen, Phenolharzen, Isocyanatharzen, Styrolharzen, Polyesterharzen, Duroplastharzen und Polycarbonatharzen ausgewählt wird.

18. Verfahren nach Anspruch 12 bis 17, wobei das Harzmaterial aus mindestens einem Epoxidharz ausgewählt wird.

19. Verfahren nach Anspruch 18, wobei das Epoxidharz ein Bisphenol-A-Harz ist.

20. Verfahren nach einem der Ansprüche 12 bis 19, wobei das Harzmaterial ferner Epichlorhydrin umfasst.

21. Verfahren nach einem der Ansprüche 12 bis 20, wobei das Harzmaterial ferner einen Füllstoff umfasst.

22. Verfahren nach Anspruch 21, wobei der Füllstoff in einer Menge von weniger als 50 % vorliegt.

23. Verfahren nach Anspruch 22, wobei der Füllstoff in einer Menge von weniger als 30 % vorliegt.

## Revendications

1. Rouleau à gaufrer gravé au laser comprenant un matériau de résine gravé au laser présentant une dureté Shore D d'au moins 90.

2. Rouleau à gaufrer selon la revendication 1, dans lequel la résine est choisie parmi au moins les résines suivantes : résines époxys, résines phénoliques, résines d'isocyanate, résines au styrène, résines polyester, résines thermodurcissables et résines de polycarbonate.

3. Rouleau à gaufrer selon la revendication 2, dans lequel le matériau de résine est choisi parmi au moins une résine époxy.

4. Rouleau à gaufrer selon la revendication 3, dans lequel la résine époxy est une résine de bisphénol A.

5. Rouleau à gaufrer selon la revendication 3 ou 4, comprenant en outre de l'épichlorhydrine de glycérol.

6. Rouleau à gaufrer selon l'une quelconque des revendications 1 à 5, comprenant en outre une matière de remplissage.

7. Rouleau à gaufrer selon la revendication 6, dans lequel la matière de remplissage est présente dans une quantité inférieure à 50%.

8. Rouleau à gaufrer selon la revendication 7, dans lequel la matière de remplissage est présente dans une quantité inférieure à 30%.

9. Rouleau à gaufrer selon l'une quelconque des revendications précédentes, dans lequel le matériau de résine forme à la fois la surface et le coeur du rouleau.

10. Rouleau à gaufrer selon l'une quelconque des revendications précédentes, dans lequel le matériau de résine forme la surface du rouleau et dans lequel le rouleau contient un coeur rigide en un autre matériau.

11. Rouleau à gaufrer selon la revendication 10, dans lequel le coeur est en acier.

12. Procédé de production d'un rouleau à gaufrer gravé au laser comprenant :
la fourniture d'un rouleau présentant une surface d'un matériau de résine pouvant être gravé au laser qui fournira une dureté Shore D d'au moins 90 pour le rouleau final ; et
la gravure au laser du matériau de résine pour établir un modèle de gaufrage dans la surface.

13. Procédé selon la revendication 12, comprenant en outre le thermodurcissage ou la cuisson du matériau de résine après l'établissement du modèle de gaufrage.

14. Procédé selon la revendication 12 ou 13, dans lequel la surface de résine est formée sur un coeur en acier.

15. Procédé selon la revendication 14, dans lequel la surface de résine est produite par revêtement au trempé, coulage ou vulcanisation.

16. Procédé selon la revendication 14 ou 15, dans lequel le coeur en acier est traité par un ou plusieurs prétraitements suivants : décapage au jet de sable, sablage ou prétraitement chimique avant de fournir la surface de résine sur le coeur.

17. Procédé selon l'une quelconque des revendications 12 à 16, dans lequel la résine est choisie parmi au moins les résines suivantes : résines époxys, résines phénoliques, résines d'isocyanate, résines au styrène, résines polyester, résines thermodurcissables et résines de polycarbonate.

18. Procédé selon l'une quelconque des revendications 12 à 17, dans lequel le matériau de résine est choisi parmi au moins une résine époxy.

19. Procédé selon la revendication 18, dans lequel la résine époxy est un résine de bisphénol A.

20. Procédé selon l'une quelconque des revendications 12 à 19, le matériau de résine comprenant en outre de l'épichlorhydrine de glycérol.

21. Procédé selon l'une quelconque des revendications 12 à 20, le matériau de résine comprenant en outre une matière de remplissage.

22. Procédé selon la revendication 21, dans lequel la matière de remplissage est présente dans une quantité inférieure à 50%.

23. Procédé selon la revendication 22, dans lequel la matière de remplissage est présente dans une quantité inférieure à 30%.
